

Oct. 15, 1946.

T. S. CARSWELL

2,409,252

CONTAINER

Filed Nov. 7, 1941



*Fig. 1.*



*Fig. 2.*

INVENTOR  
*Thomas S. Carswell*

BY

*S. M. Evans*

ATTORNEY

## UNITED STATES PATENT OFFICE

2,409,252

## CONTAINER

Thomas S. Carswell, Longmeadow, Mass., assignor  
to Monsanto Chemical Company, St. Louis, Mo.,  
a corporation of Delaware

Application November 7, 1941, Serial No. 418,231

2 Claims. (Cl. 154—43.5)

1

This invention relates to containers having a novel inner liner in combination with walls having a self-sealing structure capable of sealing a hole made therein as by such a projectile as a bullet, and more particularly pertains to a self-sealing gasoline tank, especially suitable for a military airplane, having a novel inner liner in combination with the self-sealing means.

The construction of such a tank as one suitable for a military airplane, for example, which will be not only self-sealing when punctured or traversed as by such a projectile as a bullet but also otherwise satisfactory as a tank for such motor fuel as gasoline has long presented a very difficult problem. When a high velocity bullet passes through a tank containing a liquid such as gasoline, a pressure wave is set up in the liquid as the bullet passes through it creating a liquid hammer or ram effect against the opposite wall of the tank from which the bullet entered. The result of this is a tendency to tear out a large hole where the bullet leaves the tank. This creates a special problem in constructing a self-sealing tank subject to being traversed or punctured by a bullet, since, in addition to overcoming the tendency described above, such a tank must also be otherwise satisfactory for the purpose intended.

The kind of a container to which this invention particularly relates is a self-sealing gasoline tank, which may, for example, have walls comprising, from the outside toward the inside, a layer of very heavy hide leather, a layer of latex approximately  $\frac{1}{8}$  inch thick, a layer of sponge rubber about  $\frac{1}{4}$  inch thick, another layer of latex about  $\frac{1}{8}$  inch thick, a layer of split hide, and an inner liner which is contacted by the gasoline. The inner liner serves to retain or hold the gasoline, and the other layers serve as a support and as a self-sealing means when the wall is traversed by a bullet. When a bullet passes through such a wall properly constructed in accordance with this invention, it appears that the sponge rubber tends to push into the hole to prevent substantial leakage of the gasoline, while the latex swells, when contacted by the gasoline, and expands to effect a sealing of the hole. The leather and hide impart strength and some rigidity to the tank wall.

The requirements for a satisfactory inner liner for such a container are numerous and exacting. Such a liner must not only cooperate with the self-sealing means in its function but also must serve as a satisfactory retainer for the contents, such as gasoline, of the container. Among the

chief disadvantages of prior art materials used for inner liners of containers of the kind referred to above are that such material was subject to corrosion, or was deteriorated by the substances such as gasoline placed in the container, that the material would allow gasoline to be diffused therethrough to the outer layers of the tank wall at an undesirably high rate, that the material would permit extraction of substances by the contents of the container which would contaminate the contents rendering them unsuitable for the purpose intended (gasoline, for example, might be contaminated so as to be harmful to the motor when used as motor fuel) that when traversed by a bullet the liner would be shattered, thus exposing the outer layers of the tank walls to the contents of the tank, or that the material of the liner after being traversed by the bullet, especially from the inside toward the outside accompanied by the liquid hammer or ram effect, would be expanded or torn out in such a way as to hold open the hole left by the bullet by expanded protruded portions extending into the hole so that the self-sealing means could not function properly. Although one kind of a material might be more or less satisfactory so far as many of the requirements are concerned, it would nevertheless have sufficient disadvantage to render the container highly unsatisfactory in some particular respect. For example, even though a thin sheet of aluminum might be more or less satisfactory so far as many of the requirements are concerned, it has the outstanding disadvantage that the liquid ram effect, referred to above, usually leaves a large hole torn in the sheet with portions protruding into the hole preventing the functioning of the self-sealing means. Moreover, other materials, for example, numerous synthetic materials, even though satisfactory to some extent with regard to one or some of the requirements, are unsatisfactory as to other important factors.

It is an object of this invention to provide a self-sealing container which avoids the foregoing disadvantages.

It is a further object of this invention to provide a self-sealing container having a novel inner liner in combination with the outer wall structure including the self-sealing means which improves the container.

Another object of this invention is to provide an improved self-sealing motor fuel tank especially suitable for military airplanes subject to puncture by such a projectile as a bullet.

Further and important objects of this inven-

tion will be apparent from the description which follows.

According to the present invention the significant discovery has been made that polyvinyl acetal resins give surprising satisfactory results when used in making the inner liner of such a container having a self-sealing wall structure, especially a container or tank for such hydrocarbons as gasoline, benzene, lubricating oil, etc. The polyvinyl acetal resins described in U. S. Letters Patent to Morrison et al., Reissue No. 20,430, issued June 29, 1937, and in French Patent No. 793,175 exemplify resins suitable for the purpose of this invention.

These resinous compositions are tough, elastic and flexible, and an inner liner made in accordance with this invention cooperates with the rest of the wall structure, including the self-sealing means, to produce remarkably improved results in a self-sealing container, especially a gasoline tank for a military airplane, for example.

The liners made in accordance with this invention do not corrode, as metals, for example, are resistant to deterioration by water or such contents as hydrocarbons including gasoline, benzene, lubricating oils, etc., have a surprisingly low average rate of diffusion therethrough by such materials as gasoline, do not permit extraction of substances by hydrocarbons which would contaminate the contents of the container, especially such hydrocarbons as gasoline, benzene, lubricating oil, for example, are tough, elastic and flexible and cooperate with the outer wall layers, which include the self-sealing means, to make it possible to make a wall such that, even a high speed bullet passing through the liquid contents and out through the wall accompanied by the liquid hammer or ram effect, produces only such a hole as can readily be sealed by the self-sealing means.

In order to illustrate and exemplify this invention, one embodiment thereof will be described in connection with the accompanying drawing, but it is to be understood that my invention is not necessarily limited thereto and that this embodiment is presented principally by way of illustration and exemplification of this invention and not limitation. In the drawing, Fig. 1 shows a tank constructed in accordance with this invention, and Fig. 2 shows the layers of the wall structure in detail.

A tank is shown generally at 1 and the wall thereof at 2. Referring more particularly to Fig. 2, the outer layer of the wall is shown at 3 and this may comprise a tough wear-resistant material such as a rubber impregnated rayon, for example. Layers 4 and 6 comprise a material which swells and expands when contacted by the contents of the container to effect a sealing of a hole left as by a projectile, and for such hydrocarbons as gasoline, benzene and lubricating oils, for example, especially gasoline, a material such as latex is satisfactory. At 5 is a layer of such a material as vulcanized rubber which adds elasticity to the wall structure as a whole, and appears to cushion the shock of a high speed projectile. The inner lining is shown at 7 and comprises a polyvinyl acetal resin in accordance with this invention.

It is to be understood that other outer layers of wall structure may be used in combination with the novel inner liner of this invention, but that for a self-sealing container it is highly desirable that such outer layers include an element effective to seal a hole made by a projectile and that the outer layers be such that the wall struc-

ture as a whole is sufficiently strong, elastic and non-tearing that a projectile passing therethrough leaves a hole having a sufficiently small opening that the sealing means can function properly.

The inner liner 7 comprising the polyvinyl acetal is preferably in the form of a relatively thin sheet of such a resin. It may, however, with some advantage comprise a coating of such a resin applied to the inner surface of the outer layers, and, moreover, may be made by coating or impregnating such a supporting material as duck, plywood or veneer, or by laminating a thin film of the resin to such a supporting material. As pointed out above, however, a thin sheet of the resinous material is preferred, since this makes it possible to obtain greater advantages from this material in accordance with this invention.

The polyvinyl acetals for use in accordance with this invention may be made by the polymerization of vinyl acetate or other vinyl esters, followed by saponification and reaction with an aldehyde. These esters may be polymerized to various degrees and under different conditions before hydrolysis and reaction with the aldehyde. Moreover, the resulting acetals may contain different proportions of ester, hydroxyl and acetal groups corresponding to the degree of hydrolysis and acetalization of the polymerized ester. It is desirable to select those polyvinyl acetal resins which are least affected or substantially unaffected by the contents of the container; for example, for a gasoline tank, it is desirable to use those polyvinyl acetal resins which are gasoline insoluble or the least affected by gasoline.

Polyvinyl formaldehyde acetals, such as disclosed in the patents referred to above, for example, are especially suitable. Usually the polyvinyl formals will be made by polymerizing the vinyl ester to such a degree that a one-molar solution of the polymer in benzene has a viscosity of from about 10 to 100 centipoises at 20° C., hydrolyzing and reacting such polymer with formaldehyde to produce a polyvinyl formal resin having from substantially none to about 33 per cent acetate calculated as polyvinyl acetate and from about 5 to about 15 per cent hydroxyl calculated as polyvinyl alcohol, by weight, and the rest substantially acetal. In general it is desirable to use a resin having a hydroxyl content greater than about 5 per cent and an acetate content less than about 15 per cent. Thus, such a polyvinyl formal resulting from the polymerization of vinyl acetate and hydrolysis and reaction of the polyvinyl acetate with formaldehyde to form a polyvinyl formaldehyde acetal resin containing substantially 4 to 10% hydroxyl groups calculated as polyvinyl alcohol, 9.5 to 13% acetate by weight, calculated as polyvinyl acetate, and the rest substantially acetal, is an example of a polyvinyl acetal suitable for the present invention.

For a high resistance to hydrocarbons, such as gasoline and benzene, it is preferred to use a polyvinyl formal resin in general that has a relatively low acetate content, preferably below about 10%, a relatively high hydroxyl content, preferably above about 10%, but not so high as to render the material subject to deterioration by water have been found especially desirable because of the high resistance to such hydrocarbons as gasoline or benzene, such as, for example, a polyvinyl formal having 14.6% hydroxyl calculated as polyvinyl alcohol and 1.5% acetate,

and a polyvinyl formal having a 13.4% hydroxyl content and a 8.7% acetate content.

As another example, a polyvinyl acetal suitable for this invention results from the polymerization of vinyl acetate to such a degree that a one-molar solution of the polymer in benzene had a viscosity of substantially 25 centipoises at 20° C., and the hydrolysis and reaction of the polyvinyl acetate with butyraldehyde to form a polyvinyl acetal resin containing substantially 17 to 21 per cent hydroxyl groups calculated as polyvinyl alcohol, 3% or less acetate by weight and the rest acetal.

Moreover, this invention comprehends the use of other aldehydes, such as acetaldehyde, or mixtures thereof, or even ketones in making suitable polyvinyl acetals to be used in accordance with this invention. Thus, for example, acetaldehyde, propionaldehyde, valeraldehyde, and hexaldehyde may be used. In general it is desirable to use a resin which will not be deteriorated to any substantial extent by the contents of the container, and in the case of such a hydrocarbon as gasoline or benzene, an acetal made with such lower aldehydes as formaldehyde or butyraldehyde is preferred.

The film or sheet of polyvinyl acetal for this invention may be made by any of the known methods of forming such a resin into a film or sheet, which should, of course, be non-porous for a fluid container. The resin may be extruded by means of suitable apparatus to produce a sheet, or a solution of the resin in a suitable solvent may be cast in any well-known manner and a film or sheet formed by evaporation of the solvent. Sheets of any desired thickness may be formed by these methods and a thickness of about .025 inch is usually suitable.

In general, depending on such factors as the use which is to be made of the container, for example, other resinous materials such as cellulose acetate, cellulose triacetate, the copolymer of styrene with butadiene, ethyl cellulose and other

cellulose esters may be used instead of the polyvinyl acetal resins as disclosed above.

The resinous materials used for the purpose of this invention may be plasticized, if desired, and in general most of the usual plasticizers may be used. For the polyvinyl acetal resins, and especially the polyvinyl formal resins, this invention comprehends the use of such plasticizers as, for example, diethyl phthalate, diacetin, dimethyl phthalate, dimethoxy ethyl phthalate, ethyl ethoxy ethyl phthalate, triacetin, methyl or ethyl phthalyl ethyl glycolate, triethylene glycol dibutyrate, diethylene glycol dipropionate, triethylene glycol dihexoate, dibutyl and dimethyl sebacate, triethylene glycol esters of cocoanut oil acids, and others.

What I claim is:

1. In a gasoline container characterized by the ability to self-seal when in contact with gasoline after the passage of a bullet therethrough, a wall having a layer of rubber-impregnated rayon, a layer of latex, a layer of vulcanized rubber, another layer of latex and an inner layer comprising a plasticized sheet of polyvinyl formal resin containing by weight from about 5 to 15% hydroxyl groups calculated as polyvinyl alcohol and from about 0 to 15% acetate groups calculated as polyvinyl acetate and the rest substantially acetal.
2. In a gasoline container characterized by the ability to self-seal when in contact with gasoline after the passage of a bullet therethrough, a wall having a layer of rubber-impregnated rayon, a layer of latex, a layer of vulcanized rubber, another layer of latex and an inner layer comprising a plasticized sheet of polyvinyl formal resin containing by weight from about 4 to 10% hydroxyl groups calculated as polyvinyl alcohol and from about 9.5 to 13% acetate groups calculated as polyvinyl acetate and the balance substantially acetal.

THOMAS S. CARSWELL.